

# United States Patent [19]

Yagihara et al.

[11] Patent Number: 4,892,811

[45] Date of Patent: Jan. 9, 1990

[54] SILVER HALIDE PHOTOGRAPHIC MATERIAL

[75] Inventors: Morio Yagihara; Mitsunori Ono; Akihiko Ikegawa, all of Kanagawa, Japan

[73] Assignee: Fuji Photo Film Co., Ltd., Kanagawa, Japan

[21] Appl. No.: 121,242

[22] Filed: Nov. 16, 1987

Related U.S. Application Data

[63] Continuation of Ser. No. 788,198, Oct. 16, 1985, abandoned.

[30] Foreign Application Priority Data

Oct. 16, 1984 [JP] Japan 59-216928

[51] Int. Cl.<sup>4</sup> G03C 5/54; G03C 1/42; G03C 7/26; G03C 1/34

[52] U.S. Cl. 430/562; 430/218; 430/219; 430/222; 430/251; 430/223; 430/543; 430/559; 430/564; 430/566; 430/607; 430/611; 430/613; 430/598; 430/955; 430/957; 430/958; 430/959

[58] Field of Search 430/955, 960, 218, 219, 430/505, 566, 510, 517, 957, 564, 222, 543, 959, 598, 559, 607, 613, 611, 251, 562, 223, 958

[56] References Cited

U.S. PATENT DOCUMENTS

2,322,027 6/1943 Jelley et al. 430/552  
2,857,274 10/1958 Land et al. 430/251  
3,497,502 2/1970 Taber et al. 430/522

4,186,012 1/1980 Odenwälder et al. 430/957  
4,371,604 2/1983 Van de Sande et al. 430/955  
4,420,554 12/1983 Ohashi et al. 430/955  
4,518,685 5/1985 Yagihara et al. 430/955

Primary Examiner—Richard L. Schilling  
Attorney, Agent, or Firm—Sughrue, Mion, Zinn,  
Macpeak & Seas

[57] ABSTRACT

A silver halide photographic material which comprises a support having coated thereon a light-sensitive silver halide emulsion layer, wherein the photographic material contains a blocked photographic agent represented by the following general formula (I):



wherein A represents a photographic agent moiety which is bonded to a blocking moiety through a hetero atom, or a precursor thereof; R<sup>1</sup> represents a hydrogen atom or a substituent group; and Z represents atoms necessary to form a carboxylic ring or a heterocyclic ring. The blocked photographic agent is completely stable upon storage of the photographic material, and releases a photographic agent at a desired time upon processing of the photographic material. The blocked photographic agent also exhibits its function to a substantial degree over a wide range.

14 Claims, No Drawings

**SILVER HALIDE PHOTOGRAPHIC MATERIAL**

This is a continuation of application Ser. No. 06/788,198, filed October 16, 1985, abandoned.

**FIELD OF THE INVENTION**

The present invention relates to a silver halide photographic material and, more particularly, to a silver halide photographic material containing a precursor compound of a photographically useful agent in which the active group is blocked.

**BACKGROUND OF THE INVENTION**

The manner of prior incorporation of photographically useful agents in a photographic light-sensitive material to fully achieve the effects of the agents differs from the manner in which they are used in processing solutions. For instance, photographic agents of the kind which cannot withstand long range storage in processing solutions because of their liability to decomposition under acid-alkaline or oxidation-reduction conditions can be utilized effectively and at the same time, the composition of a processing solution can be simplified to facilitate the preparation thereof. Further, in processing a light-sensitive material, it becomes feasible for a desired photographic agent to fulfill its function at a desired time and/or at a desired place, that is to say, only in a specific layer or layers in the vicinity thereof where the light-sensitive material has a multilayer structure, or for a desired photographic agent to be present in such an amount as to vary as a function of silver halide development. However, if the photographic agent is added to a photographic material in an active form, it undergoes reactions with other components present in the photographic light-sensitive material or decomposes under the influence of heat or oxygen during storage prior to processing. Therefore, it becomes impossible to achieve fully the expected capabilities at the time of processing. One solution to this problem is a method in which a photographic agent is converted into a substantially inactive form by blocking the active group, that is, a precursor thereof, and then the precursor is added to a photographic light-sensitive material. When the useful photographic agent is a dye, a functional group having a great effect on spectral absorption of the dye is blocked and, thereby, its spectral absorption is shifted to the shorter or the longer wavelength side. Under this circumstance, even if the blocked dye is also present in a silver halide emulsion layer with a spectral sensitivity in the wave-length region corresponding to the spectral absorption of the original dye, a lowering of sensitivity due to the so-called filter effect does not occur. Therefore, it can be used advantageously. When the photographically useful agent is an antifoggant or a development inhibitor, blocking of the active group can offer many advantages, e.g., desensitization due to adsorption onto light-sensitive silver halide grains and formation of silver salts upon storage can be inhibited, and at the same time, through timely release of such photographic agents, fog can be reduced without impairing photographic speed, fog arising from overdevelopment can be stopped at a desired time, and so on. When the photographically useful agent is a developer, an auxiliary developer or a fogging agent, blocking the active group or the adsorptive group can offer the advantages that various photographically adverse effects due to conversion into semiquinones or

oxidants through air oxidation on storage can be prevented, or injection of electrons into silver halides can be prevented from occurring during storage. Thereby, generation of fog nuclei can be inhibited. This results in the realization of stable processing, and the like. When the photographically useful agent is a bleach accelerator or a bleach-fix accelerator, blocking the active group can offer the advantages that in storing the light-sensitive material, reactions with other components present together with such an agent can be suppressed, while in processing it, the expected ability can be brought into full play upon removal of the blocking group at the time needed. In the present invention the above described active group, functional group and adsorptive group are generally referred to as active group.

As described above, to use a photographic agent in the form of a precursor thereof turns out to be an extremely effective means of freely achieving the ability of the photographic agent. However, precursors thereof have very severe requirements for practical use. That is, they must satisfy two contradictory requirements; one is ensuring stable presence of the precursor under a storage condition, and the other is ensuring rapid and highly efficient release of the photographic agent by removal of the blocking group at a desired time upon processing.

Several techniques for blocking photographic agents are already known. For example, well known techniques involve utilization of a blocking group such as an acyl group, a sulfonyl group or the like, as described in Japanese Patent Publication No. 44805/72 (corresponding to U.S. Pat. No. 3,615,617); utilization of a blocking group which releases a photographic agent due to the so-called reverse Michael's reaction, as described in Japanese Patent Publication Nos. 39727/79 (corresponding to U.S. Pat. No. 3,674,478), 9696/80 (corresponding to U.S. Pat. No. 3,791,830), and 34927/80 (corresponding to U.S. Pat. No. 4,009,029); utilization of a blocking group which releases a photographic agent by an intramolecular electron transfer accompanying the production of quinone methide or the analogues thereof, as described in U.S. Pat. No. 4,350,754, Japanese Patent Publication No. 39727/79, and Japanese Patent Application (OPI) Nos. 135944/82, 135945/82 and 136640/82 (the term "OPI" as used herein refers to a "published unexamined Japanese patent application"); utilization of the intramolecular ring closure reaction described in Japanese Patent Application (OPI) No. 53330/80 (corresponding to U.S. Pat. No. 4,310,612); utilization of the cleavage of a 5- or 6-membered ring described in Japanese Patent Application (OPI) Nos. 76541/82 (corresponding to U.S. Pat. No. 4,335,200), 135949/82 and 179842/82; and so on.

However, photographic agents blocked using these known techniques have the disadvantages that, for example, some precursors which are stable under storage conditions release photographic agents too slowly at the time of processing and, therefore, they require the processing under high alkalinity of a pH of 12 or above, some precursors which have sufficiently high release speeds at the time of processing under mild conditions of a pH of 9 to 11 decompose slowly under storage conditions, thereby impairing their function as a precursor, some precursors which allow little latitude in controlling the release speed at the time of processing require a very narrow pH range for effecting the processing, and so on.

## SUMMARY OF THE INVENTION

Therefore, an object of the present invention is to provide a precursor of a photographic agent which is completely stable under storage conditions and can release the photographic agent at a desired time upon processing.

Another object of the present invention is to provide a precursor of a photographic agent which can exhibit its function to a substantial degree over a wide pH range.

These objects of the present invention are attained with a silver halide photographic material which comprises a support having coated thereon a light-sensitive silver halide emulsion layer, wherein the photographic material contains at least one blocked photographic agent represented by the following general formula (I):



wherein A represents a photographic agent moiety which is bonded to a blocking moiety through a hetero atom, or a precursor thereof; R<sup>1</sup> represents a hydrogen atom or a substituent group; and Z represents atoms necessary to form a carbocyclic ring or a heterocyclic ring.

## DETAILED DESCRIPTION OF THE INVENTION

In the foregoing general formula (I), A is preferably a group represented by the general formula (II):



wherein B represents a photographic agent moiety which is bonded to X through a hetero atom contained in B; X represents a divalent linkage group which is bonded to a blocking moiety through a hetero atom contained in X; and m is 0 or 1.

Useful photographic agents, a monovalent residue of which is represented by B in the foregoing general formula (II), are known photographic agents which have at least one hetero atom and enter into combination with the blocking moiety through the hetero atom. Specific examples of such photographic agents which can be employed in the present invention include anti-foggants and development inhibitors, such as mercaptotetrazoles, mercaptotriazoles, mercaptopyrimidines, mercaptobenzimidazoles, mercaptimidazoles, mercaptobenzoxazoles, mercaptobenzthiazoles, mercaptothiadiazoles, benzotriazoles, indazoles and the like; developing agents such as p-phenylenediamines, hydroquinones, p-amino-phenols and so on; auxiliary developing agents such as pyrazolidones; fogging agents such as hydrazines, hydrazides and so on; silver halide solvents such as hypo (i.e., sodium thiosulfate) and so on; bleach accelerating agents such as aminoalkylthiols and so on; and dyes such as azo dyes, azomethine dyes and so on. In addition, photographic agents of the kind which further possess a redox function as to enable the release of the photographic agents as described above as a function of silver halide development, for example, coloring materials for color diffusion transfer photo-

graphic materials and DIR (development inhibitor releasing) hydroquinones, can also be employed as useful photographic agents.

The above described useful photographic agents may be bonded directly (when m=0 in the general formula (II)) to the blocking moiety through their hetero atom, or may be bonded via X (when m=1 in the general formula (II)) to the blocking moiety.

X represents a divalent linkage group, and it is bonded to the blocking moiety through a hetero atom contained therein. The bond formed between X and the blocking moiety is cleaved upon processing, and the resulting X-B splits per se rapidly to release a photographic agent corresponding to B. Specific examples of linkage groups of the above described kind include those which release B upon an intramolecular ring closing reaction, as described in Japanese Patent Application (OPI) No. 145135/79 (corresponding to U.S. Pat. No. 4,248,962 and British Patent Application No. 2,010,818A); those which release B by an intramolecular electron transfer, as described in British Pat. No. 2,072,363, Japanese Patent Application (OPI) No. 154234/82, U.S. Pat. Nos. 4,409,323 and 4,421,845 and so on; those which release B by elimination of carbon dioxide, as described in Japanese Patent Application (OPI) No. 179842/82 and so on; and a divalent timing group of formula  $-\text{OCH}_2-$  which releases B upon elimination of formaldehyde as described in Japanese Patent Application No. 203446/82 (corresponding to U.S. Pat. No. 4,522,917); and so on.

Representative examples of the above described linkage groups suitable for X have the structural formulae illustrated below, respectively.



wherein  $-(B)$  represents a bond to the photographic agent moiety.

More specifically, in the general formula (I), R<sup>1</sup> represents a hydrogen atom, an alkyl group (preferably containing 1 to 20 carbon atoms), an alkenyl group (preferably containing 2 to 20 carbon atoms), an aryl group (preferably containing 6 to 20 carbon atoms) or so on. These groups each may be substituted further.

Specific examples of the substituent groups include a halogen atom (e.g., a fluorine atom, a chlorine atom, a bromine atom, etc.), an alkyl group (preferably containing 1 to 20 carbon atoms), an aryl group (preferably containing 6 to 20 carbon atoms), an alkoxy group (preferably containing 1 to 20 carbon atoms), an aryloxy group (preferably containing 6 to 20 carbon atoms), an alkylthio group (preferably containing 1 to 20 carbon atoms), an arylthio group (preferably containing 6 to 20 carbon atoms), an acyl group (preferably containing 2 to 20 carbon atoms), an acylamino group (preferably an alkanoylamino group containing 1 to 20 carbon atoms or a benzoylamino group containing 6 to 20 carbon atoms), a nitro group, a cyano group, an oxycarbonyl group (preferably an alkoxy carbonyl group containing 1 to 20 carbon atoms as the alkyl moiety or an aryloxycarbonyl group containing 6 to 20 carbon atoms as the aryl moiety), a hydroxy group, a carboxy group, a sulfo group, a ureido group (preferably an alkylureido group containing 1 to 20 carbon atoms as the alkyl moiety or an arylureido group containing 6 to 20 carbon atoms as the aryl moiety), a sulfonamido group (preferably an alkylsulfonamido group containing 1 to 20 carbon atoms or an arylsulfonamido group containing 6 to 20 carbon atoms), a sulfamoyl group (preferably an alkylsulfamoyl group containing 1 to 20 carbon atoms or an arylsulfamoyl group containing 6 to 20 carbon atoms), a carbamoyl group (preferably an alkylcarbamoyl group containing 1 to 20 carbon atoms as the alkyl moiety or an arylcarbamoyl group containing 6 to 20 carbon atoms as the aryl moiety), an acyloxy group (preferably containing 1 to 20 carbon atoms), an amino group (including an unsubstituted amino group and preferably a secondary or tertiary amino group substituted with an alkyl group containing 1 to 20 carbon atoms or an aryl group containing 6 to 20 carbon atoms), a carbonic acid ester group (preferably an alkyl carbonic acid ester the alkyl moiety of which has from 1 to 20 carbon atoms or an aryl carbonic acid ester the aryl moiety of which has from 6 to 20 carbon atoms), a sulfone group (preferably an alkylsulfone group containing 1 to 20 carbon atoms or an arylsulfone group containing 6 to 20 carbon atoms), and a sulfinyl group (preferably an alkylsulfinyl group containing 1 to 20 carbon atoms or an arylsulfinyl group containing 6 to 20 carbon atoms).

The ring formed with Z include, for example, a 5-, 6- or 7- membered carbocyclic ring, a 5-, 6- or 7-membered heterocyclic ring which contains one or more hetero atoms such as nitrogen, oxygen, sulfur, etc., or a ring formed by fusing together a carbocyclic or heterocyclic ring and another ring at appropriate sites. Specific examples of such rings include cyclopentanone, cyclohexanone, cycloheptanone, benzocycloheptanone, benzocyclopentanone, benzocyclohexanone, 4-tetrahydropyridone, 4-dihydroquinolone, 4-tetrahydro-pyrene and so on.

These carbocyclic and heterocyclic rings may be substituted with one or more substituent groups, and when two or more substituent groups are present they may be the same or different.

Specific examples of substituent groups which the above described rings may have include a halogen atom (e.g., a fluorine atom, a chlorine atom, a bromine atom, etc.), an alkyl group (preferably containing 1 to 20 carbon atoms), an aryl group (preferably containing 6 to 20 carbon atoms), an alkoxy group (preferably containing 1 to 20 carbon atoms), an aryloxy group (preferably containing 6 to 20 carbon atoms), an alkylthio group

(preferably containing 1 to 20 carbon atoms), an arylthio group (preferably containing 6 to 20 carbon atoms), an acyl group (preferably containing 2 to 20 carbon atoms), an acylamino group (preferably an alkanoylamino group containing 1 to 20 carbon atoms or a benzoylamino group containing 6 to 20 carbon atoms), a nitro group, a cyano group, an oxycarbonyl group (preferably an alkoxy carbonyl group containing 1 to 20 carbon atoms as an alkyl moiety or an aryloxycarbonyl group containing 6 to 20 carbon atoms as an aryl moiety), a hydroxy group, a carboxy group, a sulfo group, a ureido group (preferably an alkylureido group containing 1 to 20 carbon atoms as an alkyl moiety or an arylureido group containing 6 to 20 carbon atoms as an aryl moiety), a sulfonamido group (preferably an alkylsulfonamido group containing 1 to 20 carbon atoms or an arylsulfonamido group containing 6 to 20 carbon atoms), a sulfamoyl group (preferably an alkylsulfamoyl group containing 1 to 20 carbon atoms or an arylsulfamoyl group containing 6 to 20 carbon atoms), a carbamoyl group (preferably an alkylcarbamoyl group containing 1 to 20 carbon atoms as an alkyl moiety or an arylcarbamoyl group containing 6 to 20 carbon atoms as an aryl moiety), an acyloxy group (preferably containing 1 to 20 carbon atoms), an amino group (including an unsubstituted amino group and preferably a secondary or tertiary amino group substituted with an alkyl group containing 1 to 20 carbon atoms or an aryl group containing 6 to 20 carbon atoms), a carbonic acid ester group (preferably an alkyl carbonic acid ester the alkyl moiety of which has from 1 to 20 carbon atoms or an aryl carbonic acid ester the aryl moiety of which has from 6 to 20 carbon atoms), a sulfone group (preferably an alkylsulfone group containing 1 to 20 carbon atoms or an arylsulfone group containing 6 to 20 carbon atoms), and a sulfinyl group (preferably an alkylsulfinyl group containing 1 to 20 carbon atoms or an arylsulfinyl group containing 6 to 20 carbon atoms).

The above described alkyl, alkenyl and aryl groups respectively include those which are further substituted with one or more of a wide variety of substituent groups as set forth above.

Further, the substituent R<sup>1</sup> is selected depending upon the pH value and the composition of the processing solution to be used for processing the photographic element in which the precursor of the photographic agent according to the present invention is incorporated, and upon the time required for timing.

More specifically the blocked photographic agent represented by the foregoing general formula (I) can be represented by the general formula (III):



wherein B represents a photographic agent moiety which is bonded to X through a hetero atom contained in B; X represents a divalent linkage group which is bonded to a blocking moiety through a hetero atom contained in X; m is 0 or 1; R<sup>1</sup> represents a hydrogen atom or a substituent group such as an alkyl group, an alkenyl group, an aryl group and the like; and Z represents atoms necessary to form a carbocyclic ring or a hetero-cyclic ring.

In addition to selection of pH of the processing solution, it becomes feasible to control the releasing speed of the photographic agent over a wide range by using a nucleophilic substance, especially sulfite ion, hydroxylamine, thiosulfate ion, metabisulfite ion or hydroxamic acid. Such nucleophilic substance is used in an amount

of about  $10^2$  to  $10^6$  mol per mol of the precursor of a photographic agent for achieving the purpose.

Specific examples of the useful precursors of photographic agents which are blocked in accordance with the present invention are illustrated below. However, the present invention should not be construed as being limited to the following examples.



(1)



(2)



(3)



(4)



(5)



(6)



-continued

(7)



(8)



(9)



(10)



(11)



(12)



(13)

-continued



(14)



(15)



(16)



(17)



(18)



(19)



(20)

-continued

(21)



(22)



(23)



(24)



(25)



(26)



-continued



(27)



(28)



(29)



(30)



(31)

-continued

(32)



Typical synthesis examples of the blocked photographic agent to be employed in the present invention are illustrated below.

#### SYNTHESIS EXAMPLE 1

##### Synthesis of Compound (1)



20 2-phenylmercapto-tetrazole and 40 g (0.4 mol) of triethylamine were dissolved in 500 ml of dry tetrahydrofuran. The reaction mixture was stirred for 4 hours at room temperature. Thereafter, tetrahydrofuran was distilled away under reduced pressure and then water was added to the reaction mixture. The resulting aqueous mixture was extracted repeatedly with ethyl acetate. The organic phase was washed with water and dried. Then, the organic solvent was distilled away under reduced pressure and thereby 61 g of crude crystals were obtained. These were recrystallized twice from an ethyl acetate-hexane mixture to yield 48 g of the desired Compound (1) as white crystals. Melting Point: 152° to 155° C.

#### SYNTHESIS EXAMPLE 2

##### Synthesis of Compound (17)



20 g (0.2 mol) of cyclohexanone and 16 g (0.2 mol) of ethyl formate were dissolved in 400 ml of dry ether, and cooled in an ice bath. To the cooled solution was added 16 g (0.4 mol) of NaH (concentration: 60%) over a 1 hour period. After the addition was concluded, the stirring was continued at room temperature for 6 hours. The reaction mixture (B in the foregoing reaction scheme precipitated) was kept cooling in an ice bath and thereto 150 ml of an ether solution containing 27 g (0.2 mol) of PCl3 was added dropwise. After the conclusion of dropwise addition, the stirring was continued at room temperature for 3 hours. The crystals thus deposited were filtered out under reduced pressure. The mother liquor was concentrated to yield 31 g of an oily substance. The oily substance was dissolved in 200 ml of dry tetrahydrofuran without purification, and added dropwise by means of a dropping funnel at room temperature into the system in which 36 g (0.2 mol) of

55 30 g (0.2 mol) of Compound B prepared in the same manner as described in the synthesis of Compound (1) was suspended in 400 ml of dry benzene and thereto phosgene gas produced from trichloromethylchloroformate (TCF) and active carbon was bubbled as the system was cooled in a water bath. After the completion of the reaction was ascertained using thin layer chromatography (it took about 1 hour for the reaction to go to completion), excess phosgene was distilled away cautiously under reduced pressure. Subsequently, benzene was distilled away under reduced pressure to obtain an oily substance (corresponding to Compound C in the foregoing reaction scheme). The oily substance was dissolved in 200 ml of dry tetrahydrofuran and cooled

in an ice bath. To the cooled solution, 150 ml of a tetrahydrofuran solution containing 25 g (0.2 mol) of N-methylaminophenol and 25 g (0.3 mol) of dry pyridine was added dropwise by slow degrees. After conclusion of dropwise addition, the stirring was continued at room temperature for an additional 4 hours. After removal of the organic solvent from the reaction mixture by distillation under reduced pressure, 400 ml of 0.5 N HCl was added thereto. The resulting mixture was extracted repeatedly with ethyl acetate. The organic phase was washed with water and dried. Then, the solvent was distilled off and thereby 58 g of a crude product was obtained. The crude product was separated and purified by passage through a chromatographic column (using an ethyl acetate-hexane (1:2) mixture as developing solvent) to yield 29 g of Compound (17) as colorless oily substance.

The precursors according to the present invention may be used in combination with two or more thereof.

The blocked photographic agents (precursors) of the present invention may be added to any constituent layers of a silver halide photographic material, including a silver halide emulsion layer, a coupler layer, a subbing layer, a protective layer, an interlayer, a filter layer, an antihalation layer, an image receiving layer, a cover sheet layer, and other auxiliary layers.

Incorporation of the precursors to be employed in the present invention into the above described layers can be carried out by adding them to coating compositions for forming the desired layers respectively as they are, or in a form of solutions prepared by dissolving in a solvent which does not adversely affect the photographic light-sensitive material, e.g., water, alcohol or the like, in appropriate concentrations. Also, the precursors can be first dissolved in high boiling point organic solvents and/or low boiling point organic solvents and further dispersed in water in the form of an emulsion and then added to the coating compositions. In addition, they may be added in such a state that they are loaded into polymer latexes using the methods as described in Japanese Patent Application (OPI) Nos. 39853/76, 59942/76 and 32552/79, U.S. Pat. No. 4,199,363 and so on.

The precursors may be added at any stage in the preparation of the photographic light-sensitive material. However, a preferable addition time is generally just before coating.

Suitable amounts of the blocked photographic agents of the present invention which can be employed depend on the kind of photographically useful agents released therefrom. Specifically, a suitable amount of an antifogant or a development inhibitor ranges from  $10^{-8}$  to  $10^{-1}$  mol per mol of silver (more specifically, that of an antifogant of the mercapto type ranges from  $10^{-6}$  to  $10^{-1}$  mol per mol of silver, and that of an antifogant of the azole type, such as benzotriazole or the like, ranges from  $10^{-5}$  to  $10^{-1}$  mol per mol of silver); that of a developing agent ranges from  $10^{-2}$  to 10 mols, preferably from 0.1 to 5 mols, per mol of silver; that of an auxiliary developing agent like a pyrazolidone ranges from  $10^{-4}$  to 10 mols, preferably from  $10^{-2}$  to 5 mols, per mol of silver; that of a fogging agent ranges from  $10^{-2}$  to  $10^{-6}$  mol, preferably from  $10^{-3}$  to  $10^{-5}$  mol, per mol of silver; that of a silver halide solvent, such as hypo or so on, ranges from  $10^{-3}$  to 10 mols, preferably from  $10^{-2}$  to 1 mol, per mol of silver; that of a bleach accelerator, such as an aminoethanethiol or so on, ranges from  $10^{-5}$  to 0.1 mol, preferably from  $10^{-4}$  to  $10^{-2}$  mol, per mol of silver; and that of dyes or coloring

agents for color diffusion transfer photographic materials, respectively, ranges from  $10^{-3}$  to 1 mol, preferably from  $5 \times 10^{-3}$  to 0.5 mol, per mol of silver.

The precursors of photographic agents to be employed in the present invention are completely stable under storage conditions and can release the photographic agent at a desired time upon processing due to their particular blocking moiety illustrated in the foregoing general formula (I).

Further, photographic light-sensitive materials containing the precursors of photographic agents in which the photographic moiety is an antifogant or a development inhibitor and the blocking moiety is in accordance with the present invention have an advantage in that the screen range is long when dot images are formed and, therefore, they are especially suitable for photographic light-sensitive materials for plate making.

The compounds of the present invention can be employed in color photographic light-sensitive materials of, e.g., the incorporated coupler type system. Specific examples of color photographic materials include color photograph-taking negative films (for amateur use, motion picture use, etc.), color reversal films, color paper, color reversal paper, cinema positive films, and so on.

Also, the compounds of the present invention can be employed in the photographic system in which positive dye images are produced according to a silver dye bleach process, as described in T. H. James (editor), *The Theory of the Photographic Process*, 4th Ed., Chap. 12, pp. 363-366 (Title: Principles and Chemistry of Color Photography IV. Silver Dye Bleach Process), Macmillan, New York (1977), and so on.

Moreover, the compounds of the present invention can be employed in black-and-white photographic materials. Specific examples of black-and-white photographic materials include direct medical X-ray films, black-and-white films for amateur use, lith films, scanner films, and so on.

In these color photographic materials and black-and-white photographic materials, the compounds of the present invention can be incorporated in any constituent layers thereof, including an emulsion layer, an interlayer, a surface protective layer and so on.

When the compounds of the present invention are applied to the color diffusion transfer process, the silver halide photographic material of the present invention can have a film unit structure of the peel-apart type; that of the integrated type as described in Japanese Patent Publication Nos. 16356/71 and 33697/73, Japanese Patent Application (OPI) No. 13040/75, and British Pat. No. 1,330,524; or that of the no peel-apart type as described in Japanese Patent Application (OPI) No. 119345/82. The precursors represented by the foregoing general formula (I) may be added to any layer of the film unit, provided that they are associated with silver halide emulsions so as to act effectively upon development of the silver halide emulsions. However, it is preferable to add them to a light-sensitive layer such as a light-sensitive silver halide emulsion-containing layer, a dye image providing compound-containing layer or other auxiliary layers; a subsidiary layer such as an image receiving layer or a white reflecting layer; or a neutralizing structure such as a neutralizing layer, a neutralization timing layer or the like. Of these layers, the neutralizing layer or the neutralization timing layer is especially desirable for addition.

It is advantageous to use gelatin as a binder or a protective colloid of emulsion layers and inter-layers to

constitute the photographic material of the present invention. Of course, other hydrophilic colloids can also be used alone or as combinations with gelatin.

In the present invention, gelatin may be either lime-processed one or acid-processed one. Details of the preparation of gelatin are described in Arthur Veis, *The Macromolecular Chemistry of Gelatin*, Academic Press (1964).

To the photographic emulsions to be used in the present invention, surface active agents may be added 10 alone or as a combination of two or more thereof.

They are, in general, used as coating aids, and occasionally for other purposes, for instance, emulsifying dispersion, improvements in photographic characteristics concerning sensitization, prevention of generation 15 of static charges, prevention of adhesion and so on. Examples of useful surface active agents include natural surface active agents such as saponin, etc.; nonionic surface active agents such as those of alkylene oxide type, those of glycerol type, those of glycidol type, etc.; cationic surface active agents such as higher alkyl amines, quaternary ammonium salts, pyridines and other heterocyclic compounds, phosphoniums, sulfoniums, etc.; anionic surface active agents containing an acidic group such as a carboxylic acid group, a sulfonic acid group, a phosphoric acid group, a sulfate group, a phosphate group, etc.; and amphoteric surface active agents such as amino acids, aminosulfonic acids, sulfates or phosphates of aminoalcohols, etc.

Suitable examples of polyalkylene oxide compounds which can be used in the present invention include products obtained by condensation reaction of polyalkylene oxides containing at least 10 units of alkylene oxide having 2 to 4 carbon atoms, for example, ethylene oxide, propylene-1,3-oxide, butylene-1,2-oxide, etc., especially ethylene oxide, with compounds having at least one active hydrogen atom, for example, water, aliphatic alcohols, aromatic alcohols, fatty acids, organic amines, hexitol derivatives, etc.; and block copolymers of two or more kinds of polyalkylene oxides. More specifically, polyalkylene glycols, polyalkylene glycol alkyl ethers, polyalkylene glycol aryl ethers, polyalkylene glycol (alkyl aryl) esters, polyalkylene glycol esters, polyalkylene glycol fatty acid amides, polyalkylene glycol amines, polyalkylene glycol block 40 copolymers, polyalkylene glycol graft copolymers and so on can be used as such polyalkylene oxide compounds. Molecular weights of these polyalkylene oxide compounds must be at least 600.

Two or more polyalkylene oxide chains may be contained in a molecule. Therein, each polyalkylene oxide chain may be composed of less than 10 alkylene oxide units, but the total alkylene oxide units in a molecule should be at least 10. Where two or more polyalkylene oxide chains are contained in a molecule, they may be composed of different alkylene oxide units, for example, ethylene oxide and propylene oxide. Polyalkylene oxide compounds which can be preferably used in the present invention are those containing from 14 to 100 alkylene oxide units.

Specific examples of polyalkylene oxide compounds which can be used in the present invention are set forth below.

P-1 HO(CH<sub>2</sub>CH<sub>2</sub>O)<sub>90</sub>H

P-2 C<sub>4</sub>H<sub>9</sub>O(CH<sub>2</sub>CH<sub>2</sub>O)<sub>15</sub>H

P-3 C<sub>12</sub>H<sub>25</sub>O(CH<sub>2</sub>CH<sub>2</sub>O)<sub>15</sub>H

P-4 C<sub>18</sub>H<sub>37</sub>O(CH<sub>2</sub>CH<sub>2</sub>O)<sub>15</sub>H

P-5 C<sub>18</sub>H<sub>37</sub>O(CH<sub>2</sub>CH<sub>2</sub>O)<sub>40</sub>H

P-6 C<sub>8</sub>H<sub>17</sub>CH=CHC<sub>8</sub>H<sub>16</sub>O(CH<sub>2</sub>CH<sub>2</sub>O)<sub>15</sub>H



P-10 C<sub>11</sub>H<sub>23</sub>COO(CH<sub>2</sub>CH<sub>2</sub>O)<sub>80</sub>H

P-11 C<sub>11</sub>H<sub>23</sub>COO(CH<sub>2</sub>CH<sub>2</sub>O)<sub>24</sub>OCC<sub>11</sub>H<sub>23</sub>



P-13 C<sub>11</sub>H<sub>23</sub>CONH(CH<sub>2</sub>CH<sub>2</sub>O)<sub>15</sub>H



P-15 C<sub>14</sub>H<sub>29</sub>N(CH<sub>2</sub>)(CH<sub>2</sub>CH<sub>2</sub>O)<sub>24</sub>H



CH<sub>3</sub>

a + b + c = 50

b:a + c = 10:9



P-20 HO(CH<sub>2</sub>CH<sub>2</sub>O)<sub>a</sub>(CH<sub>2</sub>CH<sub>2</sub>CH<sub>2</sub>CH<sub>2</sub>O)<sub>b</sub>(CH<sub>2</sub>CH<sub>2</sub>O)<sub>c</sub>H

a + c = 30, b = 14

P-21 HO(CH<sub>2</sub>CH<sub>2</sub>O)<sub>a</sub>(CHCH<sub>2</sub>O)<sub>b</sub>(CH<sub>2</sub>CH<sub>2</sub>O)<sub>c</sub>H



b = 8, a + c = 50

P-22



P-23

P-24 HO-(CH<sub>2</sub>CH<sub>2</sub>O)<sub>34</sub>-H

The polyalkylene oxide compounds illustrated above are described in Japanese Patent Application (OPI) Nos. 156423/75, 108130/77 and 3217/78. These polyalkylene oxide compounds may be used alone or in a mixture of two or more thereof.

These polyalkylene oxide compounds can be added to silver halide emulsions in the form of a solution prepared by dissolving them in water or a low boiling point organic solvent compatible with water in proper concentrations at an appropriate stage of emulsion-making prior to coating, preferably after the chemical ripening thereof. The polyalkylene oxide compounds which can be used in the present invention are added in an amount ranging preferably from  $1 \times 10^{-5}$  to  $1 \times 10^{-2}$  mol per mol of silver halide.

Silver halides which can be used in photographic emulsion layers to constitute the photographic light-sensitive material of the present invention include silver bromide, silver iodobromide, silver iodochlorobromide, silver chlorobromide and silver chloride. Of these silver halides, silver iodobromide having an iodide content of 15 mol% or less is preferred over others. Especially good results can be obtained when an iodide content in the silver iodobromide ranges from 2 to 12 mol %.

The present invention is not particularly restricted as to mean grain size of silver halide grains in the photographic emulsion layers. (The grain size herein refers to the grain diameter when the grains are spherical or approximately spherical in shape, while it refers to the edge length when the grains are cubic in shape. In both cases, it is represented by the mean based on the projected areas of grains.) However, it is preferably 3  $\mu\text{m}$  or less.

The distribution of the grain size can be either narrow or broad.

The silver halide grains in the photographic emulsions may have a regular crystal form, such as that of a cube, an octahedron or so on; an irregular crystal form, such as that of a sphere, a tabular form or so on; or a composite form thereof. A mixture of various crystal forms of silver halide grains may also be present.

Photographic emulsions in which silver halide grains having such a supertabular shape that the grain diameter is not less than five times the grain thickness are contained in a fraction of 50% or more, based on the total projected area of all grains present therein, may be employed in the present invention.

The interior and the surface of the silver halide grains may differ, and either silver halide grains of the kind which form a latent image predominantly at the surface

of the grains, or grains of the kind which mainly form a latent image inside the grains may be used.

The photographic emulsions employed in the present invention can be prepared using various methods, as described in, for example, P. Glafkides, *Chimie et Physique Photographique*, Paul Montel, Paris (1967), G. F. Duffin, *Photographic Emulsion Chemistry*, The Focal Press, London (1966), V. L. Zelikman et al, *Making and Coating Photographic Emulsion*, The Focal Press, London (1964), and so on. More specifically, the acid process, the neutral process, the ammonia process and so on can be employed. Suitable methods for reacting a water-soluble silver salt with a water-soluble halide include, for example, a single jet method, a double jet method or a combination thereof.

Also, a method in which silver halide grains are produced in the presence of excess silver ion (the so-called reversal mixing method) can be employed in the present invention. Further, the so-called controlled double jet method, in which the pAg of the liquid phase wherein silver halide grains are to be precipitated is maintained constant, may also be employed in the present invention. According to this method, silver halide emulsions having a regular crystal form and an almost uniform grain size can be obtained.

Two or more of silver halide emulsions prepared separately may be used in a form of mixture thereof.

In a process of producing silver halide grains or allowing the produced silver halide grains to ripen physically, cadmium salts, zinc salts, lead salts, thallium salts, iridium salts or complexes thereof, rhodium salts or complexes thereof, iron salts or complexes thereof and/or the like may be present.

It is usual for the silver halide emulsion of the present invention to be chemically sensitized. Chemical sensitization can be carried out using processes described in H. Frieser (editor), *Die Grundlagen der Photographischen Prozesse mit Silberhalogeniden*, pp. 675 to 734, Akademische Verlagsgesellschaft (1968), and so on.

More specifically, sulfur sensitization using active gelatin or compounds containing sulfur capable of reacting with silver ion (e.g., thiosulfates, thioureas, mercapto compounds, rhodamines and so on), reduction sensitization using reducing materials (e.g., stannous salts, amines, hydrazine derivatives, formamidine sulfonic acid, silane compounds and so on), noble metal sensitization using noble metal compounds (e.g., gold metal complexes, and Group VIII metal complexes such as those of platinum, iridium, palladium, etc.), and so on can be employed individually or as a combination thereof.

The photographic emulsion of the present invention can contain a wide variety of compounds for purposes of preventing fog or stabilizing photographic functions during production, storage, or photographic processing. Specifically, azoles such as benzothiazolium salts, nitroimidazoles, nitrobenzimidazoles, chlorobenzimidazoles, bromobenzimidazoles, mercaptobenzimidazoles, mercaptobenzothiazoles, mercaptobenzimidazoles, mercaptothiadiazoles, aminotriazoles, benzotriazoles, nitrobenzotriazoles, mercaptotetrazoles (especially 1-phenyl-5-mercaptotetrazole) and so on; mercaptopyrimidines; mercaptotriazines; thioketo compounds like oxazolidinethiones; azaindenes such as triazaindenes, tetraazaindenes (especially 4-hydroxy-substituted (1,3,3a,7)tetraazaindenes), pentaazaindenes and so on; and compounds which have been known as antifoggants or stabilizers, such as benzenethiosulfonic acid,

benzenesulfinic acid, benzenesulfonic acid amide, and so on can be added to the silver halide emulsions.

Photographic emulsions of the photographic light-sensitive material to be used in the present invention may further contain, for example, thioether compounds, thiomorpholines, quaternary ammonium salt compounds, urethane derivatives, urea derivatives, imidazole derivatives, 3-pyrazolidones and so on in order to increase the sensitivity and contrast, or in order to accelerate the developing rate thereof.

Furthermore, the photographic light-sensitive material of the present invention can contain a dispersion of water-insoluble or slightly soluble polymers in photographic emulsion layers or other hydrophilic colloid layers for the purpose of improvements in dimensional stability and so on. Suitable examples of such polymers include homopolymers or copolymers in which alkyl(-meth)-acrylates, alkoxyalkyl(meth)acrylates, glycidyl(-meth)-acrylates, (meth)acrylamides, vinyl esters (e.g., vinyl acetate), acrylonitrile, olefins, styrenes and so on are contained alone or in combinations of two or more as constitutional repeating units, and copolymers which contain a combination of one or more of the monomers set forth above and one or more of other monomers, such as acrylic acid, methacrylic acids,  $\alpha,\beta$ -unsaturated dicarboxylic acids, hydroxyalkyl(meth)acrylates, a sulfoalkyl(meth)acrylate, styrenesulfonic acid and so on, as constitutional repeating units.

The photographic emulsions to be used in the present invention may be spectrally sensitized using methine dyes or other dyes. Specific spectral sensitizing dyes which can be employed include cyanine dyes, merocyanine dyes, complex cyanine dyes, complex merocyanine dyes, holopolar cyanine dyes, hemicyanine dyes, styryl dyes and hemioxonol dyes. Especially useful dyes are cyanine dyes, merocyanine dyes and complex merocyanine dyes. Any nuclei usually present in cyanine dyes can be the basic heterocyclic nuclei of these dyes. More specifically, basic heterocyclic nuclei include pyrrolidine, oxazoline, thiazoline, pyrrole, oxazole, thiazole, selenazole, imidazole, tetrazole, pyridine and like nuclei; nuclei formed by fusing together one of the above described nuclei and an alicyclic hydrocarbon ring; and nuclei formed by fusing together one of the above described nuclei and an aromatic hydrocarbon ring. Specific examples of these nuclei include indolenine, benzindolenine, indole, benzoxazole, naphthoxazole, benzothiazole, naphthothiazole, benzoselenazole, benzimidazole, quinoline and like nuclei. Each of these nuclei may be substituted on its carbon atom.

The merocyanine dyes or the complex merocyanine dyes can contain 5- or 6-membered heterocyclic nuclei, such as pyrazolin-5-one, thiohydantoin, 2-thioxazolidin-2,4-dione, thiazolidin-2,4-dione, rhodanine, thiobarbituric acid and like nuclei, as ketomethylene structure-containing nuclei.

These sensitizing dyes may be employed individually or in combination. Combinations of sensitizing dyes are often employed for the purpose of supersensitization.

Substances which can exhibit a supersensitizing effect in combination with a certain sensitizing dye although they themselves do not spectrally sensitize silver halide emulsions or do not absorb light in the visible region may be incorporated into the silver halide emulsions. For example, aminostilbene compounds substituted with nitrogen-containing heterocyclic groups (for instance, as described in U.S. Pat. Nos. 2,933,390 and 3,635,721), aromatic organic acid-formaldehyde con-

denses (for instance, as described in U.S. Pat. No. 3,743,510), cadmium salts, azaindene compounds and so on can be employed.

The present invention can also be applied to a multi-layer multicolor photographic material having at least two photographic emulsion layers having different color sensitivities on a support. A multilayer color photographic material has, in general, at least one red-sensitive emulsion layer, at least one green-sensitive emulsion layer, and at least one blue-sensitive emulsion layer on a support. The order of these layers can be varied as desired. Usually cyan-, magenta-, and yellow-forming couplers are incorporated in red-, green-, and blue-sensitive emulsion layers, respectively. However, different combinations can be employed, if desired.

In addition to the foregoing compounds of the present invention, color forming couplers, that is to say, compounds capable of forming colors by coupling with the oxidation product of aromatic primary amine developing agents (e.g., phenylenediamine derivatives, amino-phenol derivatives, etc.) upon color development processing, can be incorporated in the same or different photographic emulsion layers, or light-insensitive layers of the photographic light-sensitive material produced in accordance with the present invention. Specific examples of magenta couplers which can be used include 5-pyrazolone couplers, pyrazolobenzimidazole couplers, pyrazoloimidazole couplers, pyrazolopyrazole couplers, pyrazolotriazole couplers, pyrazolotetrazole couplers, cyanoacetylcumarone couplers, open chain acylacetone nitrile couplers, and so on. Specific examples of yellow couplers which can be used include acylacetamide couplers (e.g., benzoylacetanilides, pivaloylacetanilides, etc.), and so on. Specific examples of cyan couplers which can be used include naphthol couplers, phenol couplers, and so on. Of these couplers, nondiffusible couplers which contain a hydrophobic group as a so-called ballast group in a molecule and polymerized couplers are more advantageous. The couplers may be either 4-equivalent or 2-equivalent with respect to silver ion. In addition, the couplers may be colored couplers having a color correcting effect, and couplers capable of releasing development inhibitors upon development (so-called DIR couplers). Besides DIR couplers, colorless DIR coupling compounds which form colorless products upon the coupling reaction and release development inhibitors can also be incorporated.

Two or more of the above described couplers and the like can be incorporated into the same layer, or the same compound can also be incorporated into two or more different layers to achieve the characteristics required of the photographic material.

The compounds of the present invention and couplers which can be used in combination therewith in the present invention can be introduced into silver halide emulsion layers using known methods as described in, e.g., U.S. Pat. No. 2,322,027. Specifically, they are dissolved in high boiling point organic solvents, such as phthalic acid alkyl esters (e.g., dibutyl phthalate, diethyl phthalate, etc.), phosphoric acid esters (e.g., diphenyl phosphate, triphenyl phosphate, tricresyl phosphate, diethyl butyl phosphate, etc.), citric acid esters (e.g., tributyl acetyl citrate, etc.), benzoic acid esters (e.g., octyl benzoate, etc.), alkylamides (e.g., diethyl lauryl amide, etc.), fatty acid esters (e.g., dibutoxyethyl succinate, diethyl azelate, etc.), trimesic acid esters (e.g., tributyl trimesate, etc.) and so on, or in low boiling

point organic solvents having boiling points ranging from about 30° C. to about 150° C., such as lower alkyl acetates (e.g., ethyl acetate, butyl acetate, etc.), ethyl propionate, secondary butyl alcohol, methyl isobutyl ketone,  $\beta$ -ethoxyethyl acetate, methyl cellosolve acetate and so on and then dispersed into hydrophilic colloids. The above described high boiling point organic solvents and low boiling point organic solvents may be employed in a form of mixture of two or more thereof.

In addition, the compounds of the present invention and the couplers can be dispersed into hydrophilic colloids using polymers described in Japanese Patent Publication No. 39853/76, and Japanese Patent Application (OPI) No. 59943/76.

When the couplers contain acidic groups such as carboxylic acid, sulfonic acid and the like, the couplers are introduced into hydrophilic colloids as alkaline aqueous solutions.

The photographic emulsion layers or other hydrophilic colloid layers which constitute the photographic material of the present invention may contain inorganic or organic hardeners. Examples of hardeners which can be used include chromium salts (e.g., chrome alum, chromium acetate, etc.), aldehyde compounds (e.g., formaldehyde, glyoxal, glutaraldehyde, etc.), N-methylol compounds (e.g., dimethylolurea, methylol-dimethylhydantoin, etc.), dioxane derivatives (e.g., 2,3-dihydroxydioxane, etc.), active vinyl compounds (e.g., 1,3,5-triacyloyl-hexahydro-s-triazine, 1,3-vinylsulfonyl-methyl-2-propanol, etc.), active halogen-containing compounds (e.g., 2,4-dichloro-6-hydroxy-s-triazine, etc.), halogeno carboxydehydes (such as mucochloric acid, mucophenoxychloric acid, etc.), and so on. These hardeners may be used alone or as a combination of two or more thereof.

When dyes, ultraviolet absorbing agents and the like are contained in hydrophilic colloid layers of the photographic material prepared in accordance with the present invention, they may be fixed inside the hydrophilic colloid layers using a mordant like a cationic polymer and so on.

The photographic material prepared in accordance with the present invention may contain as a color fog inhibitor a hydroquinone derivative, an aminophenol derivative, a gallic acid derivative, an ascorbic acid derivative and so on.

Hydrophilic colloid layers of the photographic material prepared in accordance with the present invention may contain an ultraviolet absorbing agent. For example, aryl-substituted benzotriazole compounds (e.g., those described in U.S. Pat. No. 3,533,794), 4-thiazolidone compounds (e.g., those described in U.S. Pat. Nos. 3,314,794 and 3,352,681), benzophenone compounds (e.g., those described in Japanese Patent Application (OPI) No. 2784/71), cinnamate compounds (e.g., those described in U.S. Pat. Nos. 3,705,805 and 3,707,375), butadiene compounds (e.g., those described in U.S. Pat. No. 4,045,229) and benzoxazole compounds (e.g., those described in U.S. Pat. No. 3,700,455) can be used as ultraviolet absorbing agents. Also, ultraviolet absorbing couplers (e.g., cyan dye forming couplers of the  $\alpha$ -naphthol type) and ultraviolet absorbing polymers may be used. These ultraviolet absorbing agents may be mordanted inside a particular layer.

The photographic material prepared in accordance with the present invention may contain water-soluble dyes as filter dyes, antihalation dyes or dyes for various other purposes in its hydrophilic colloid layers. Exam-

ples of dyes useful for the above described purposes include oxonol dyes, hemioxonol dyes, styryl dyes, merocyanine dyes, cyanine dyes, and azo dyes. Of these dyes, oxonol dyes, hemioxonol dyes, and merocyanine dyes are used to a greater advantage.

In the present invention, known discoloration inhibitors can be used. Color image stabilizers which can be used in the present invention can be used alone or in combinations of two or more thereof. Specific examples 10 of known discoloration inhibitors include hydroquinone derivatives, gallic acid derivatives, p-alkoxyphenols, p-oxyphenol derivatives, and bisphenols.

The present invention is not particularly restricted as to the developing method for the silver halide photographic material, and known processing methods and known processing solutions, as described, e.g., in *Research Disclosure*, Vol. 176, pp. 28-30, can be employed in the present invention. This photographic processing may be either a photographic processing for forming a silver image (black-and-white processing) or a photographic processing for forming a dye image (color photographic processing), depending upon the end-use purpose of the photographic material. The processing temperature is generally in the range of about 18° C. to 25 about 50° C. Of course, temperatures lower than about 18° C. or higher than about 50° C. may be employed.

Dye images can be formed using conventional methods. For instance, a negative-positive process (as described in *Journal of the Society of Motion Picture and Television Engineers*, Vol. 61, pp. 667-701 (1953); a color reversal process in which a negative silver image is formed by development with a developing solution containing a black-and-white developing agent, uniform exposure or another appropriate fogging treatment is 35 then carried out at least once, and subsequently color development is carried out to provide a positive dye image; a silver dye bleach process in which dye-containing photographic emulsion layers are developed after exposure to produce a silver image, and the dyes 40 are bleached using the resulting silver image as a bleaching catalyst; and so on can be employed.

A color developing solution is, in general, an alkaline aqueous solution containing a color developing agent. Suitable examples of color developing agents which can be used include known aromatic primary amine developers, such as phenylenediamines (e.g., 4-amino-N,N-diethylaniline, 3-methyl-4-amino-N,N-diethylaniline, 4-amino-N-ethyl-N- $\beta$ -hydroxyethylaniline, 3-methyl-4-amino-N-ethyl-N- $\beta$ -hydroxyethylaniline, 3-methyl-4-amino-N-ethyl-N- $\beta$ -methanesulfonamidoethylaniline, 4-amino-3-methyl-N-ethyl-N- $\beta$ -methoxyethylaniline, etc.).

In addition to the color developing agents set forth above, those described in L. F. A. Mason, *Photographic Processing Chemistry*, pp. 226-229, The Focal Press, London (1966), U.S. Pat. Nos. 2,193,015 and 2,592,364, Japanese Patent Application (OPI) No. 64933/73, and so on, may be also employed.

Besides color developing agents as described above, the color developing solution can contain a pH buffering agent such as sulfites, carbonates, borates and phosphates of alkali metals, a development inhibitor or an antifoggant such as bromides, iodides and organic antifoggants, and so on. Optionally, a water softener, a preservative such as hydroxylamines, etc., an organic solvent such as benzyl alcohol, diethylene glycol, etc., a development accelerator such as polyethylene glycols, quaternary ammonium salts, amines, etc., dye forming

couplers, competing couplers, a fogging agent such as sodium borohydride, etc., an auxiliary developer such as 1-phenyl-3-pyrazolidone, etc., a viscosity imparting agent, chelating agents of polycarboxylic acid type, an antioxidant, and so on, may be contained in the color developing solution.

The photographic emulsion layers which have been color development-processed are generally subjected to a bleach processing. The bleach processing may be carried out either simultaneously with or separately from a fix processing. Suitable examples of bleaching agents which can be used include compounds of polyvalent metals such as iron (III), cobalt (III), chromium (VI), copper (II), etc., peroxy acids, quinones, nitroso compounds, and so on.

More specifically, ferricyanides, dichromates, organic complex salts of Fe (III) or Co (III) such as complex salts of aminopolycarboxylic acids, e.g., ethylenediaminetetraacetic acid, nitrilotriacetic acid, 1,3-diamino-2-propanoltetraacetic acid, etc., or organic acids, e.g., citric acid, tartaric acid, malic acid, etc., persulfates, permanganates, nitrosophenol, and so on, can be employed as bleaching agents. Of these compounds, potassium ferricyanide, sodium ethylenediamine-tetraacetato ferrate (III), and ammonium ethylenediamine-tetraacetato ferrate (III) are especially useful. In particular, (ethylenediaminetetraacetato)iron (III) complexes are used to advantage in both an independent bleaching bath and a combined bleaching and fixing bath.

A fixing bath which can be used in the present invention includes those having generally used compositions. Therein, not only thiosulfates and thiocyanates but also organic sulfur compounds which are known to have a fixing effect can be used as fixing agents. In the fixing solution, water-soluble aluminum salts may be contained as hardeners.

The developing solution employed for black-and-white photographic processing can contain known developing agents. Suitable developing agents include dihydroxybenzenes (e.g., hydroquinone), 3-pyrazolidones (e.g., 1-phenyl-3-pyrazolidone), aminophenols (e.g., N-methyl-p-aminophenol), etc., and they can be used alone or in combination. The developing solution can generally contain, in addition to the above described developing agents, known preservatives, alkali agents, pH buffering agents and antifoggants and optionally may contain dissolving aids, color toning agents, development accelerators, surface active agents, defoaming agents, water softeners, hardeners, viscosity imparting agents and so on.

The photographic emulsions of the present invention can also be subjected to the so-called "lithographic" development processing, if desired. "Lithographic" development processing is the processing in which in order to effect the photographic reproduction of line images or the photographic reproduction of halftone images by means of dots, dihydroxybenzenes are generally used as developing agents and the development step is made to proceed infectiously under the condition that a sulfite ion concentration is maintained at a low level (the details of which are described in L.F.A. Mason, *Photographic Processing Chemistry*, pp. 163-165 (1966)).

The present invention is illustrated in greater detail by reference to the following examples, but is should not be construed as being limited to these examples.

Unless otherwise specified, all percents, ratios, etc., are by weight.

#### EXAMPLE 1

In order to evaluate the effectiveness of the photographic agents which were blocked in accordance with the present invention, Samples A to G were prepared in the manner described below, in which the compounds of the present invention and the comparison compounds corresponding thereto were employed, respectively. One of the antifoggants set forth in Table 1 or one of the corresponding thereto were employed, respectively. One of the antifoggants set forth in Table 1 or one of the blocked photographic agents (precursors) of the present invention set forth also in Table 1 was dissolved in tricresyl phosphate together with Coupler Cp-1, emulsified, and added to a silver halide emulsion. The resulting emulsion was coated on a cellulose triacetate support having a subbing layer. The coverage of each ingredient was expressed in terms of g/m<sup>2</sup> or mol/m<sup>2</sup>, and designated in parentheses.

##### (1) Emulsion Layer

Negative type silver iodobromide emulsion having a grain size of 1.4  $\mu$  m (silver:  $1.6 \times 10^{-2}$  mol/m<sup>2</sup>)

Magenta Coupler Cp-1 ( $1.33 \times 10^{-3}$  mol/m<sup>2</sup>)

Antifoggant, or precursor compound of the present invention (as shown in Table 1)

Gelatin (2.50 g/m<sup>2</sup>)

(2) Protective Layer

Gelatin (1.30 g/m<sup>2</sup>)

Sodium 2,4-dichloro-6-hydroxy-s-triazine (0.05 g/m<sup>2</sup>)

These films were allowed to stand for 14 hours under conditions of 40° C. and 70% RH. Thereafter, they were subjected to imagewise exposure for sensitometry and then to the following color development processing.

|    | Steps for Color Development Processing | Time         | Temperature |
|----|----------------------------------------|--------------|-------------|
| 40 | 1. Color Development                   | 3 min 15 sec | 38° C.      |
|    | 2. Bleaching                           | 6 min 30 sec | "           |
|    | 3. Washing                             | 2 min        | "           |
|    | 4. Fixing                              | 4 min        | "           |
|    | 5. Washing                             | 4 min        | "           |
| 45 | 6. Stabilizing                         | 1 min        | "           |

Compositions of the processing solutions employed in the above described steps, respectively, are described below.

##### Color Developing Solution:

|                                                         |             |
|---------------------------------------------------------|-------------|
| Water                                                   | 800 ml      |
| 4-(N-Ethyl-N-hydroxyethyl)amino-2-methylaniline Sulfate | 5 g         |
| Sodium Sulfite                                          | 5 g         |
| Hydroxylamine Sulfate                                   | 2 g         |
| Potassium Carbonate                                     | 30 g        |
| Potassium Hydrogencarbonate                             | 1.2 g       |
| Potassium Bromide                                       | 1.2 g       |
| Sodium Chloride                                         | 0.2 g       |
| Trisodium Nitrilotriacetate                             | 1.2 g       |
| Water to make                                           | 1 liter     |
|                                                         | (pH = 10.1) |

##### Bleaching Solution:

|                                                    |            |
|----------------------------------------------------|------------|
| Water                                              | 800 ml     |
| Ammonium Ethylenediaminetetraacetato Ferrate (III) | 100 g      |
| Disodium Ethylenediaminetetraacetate               | 10 g       |
| Potassium Bromide                                  | 150 g      |
| Acetic Acid                                        | 10 g       |
| Water to make                                      | 1 liter    |
|                                                    | (pH = 6.0) |

-continued

Fixing Solution:

|                        |                       |
|------------------------|-----------------------|
| Water                  | 800 ml                |
| Ammonium Thiosulfate   | 150 g                 |
| Sodium Sulfite         | 10 g                  |
| Sodium Hydrogensulfite | 2.5 g                 |
| Water to make          | 1 liter<br>(pH = 6.0) |

Stabilizing Solution:

|                              |        |
|------------------------------|--------|
| Water                        | 800 ml |
| Formaldehyde (37% aq. soln.) | 5 ml   |

-continued

|                                       |         |
|---------------------------------------|---------|
| Polyoxyethylene p-Mononylphenyl Ether | 0.2 g   |
| Water to make                         | 1 liter |

5

The photographic properties thus obtained are shown in Table 1.

The coupler and the antifoggants for comparison employed in the above described samples are illustrated below.

Cp-1



A-1



A-2



A-3



(Precursor described in U.S. Pat. No. 3,888,677)

TABLE 1

| Sample            | Precursor Compound<br>of the Present<br>Invention or<br>Comparison<br>Antifoggants | Amount Added<br>(mol/m <sup>2</sup> ) | Fog  |       |     | Relative*<br>Sensitivity | Maximum<br>Color<br>Density |
|-------------------|------------------------------------------------------------------------------------|---------------------------------------|------|-------|-----|--------------------------|-----------------------------|
|                   |                                                                                    |                                       |      | Gamma |     |                          |                             |
| A<br>(Control)    | —                                                                                  | —                                     | 0.12 | 0.84  | 100 | 100                      | 1.67                        |
| B<br>(Invention)  | (1)                                                                                | 1.1 × 10 <sup>-5</sup>                | 0.07 | 0.77  | 98  | 98                       | 1.59                        |
| C<br>(Invention)  | (3)                                                                                | 1.1 × 10 <sup>-5</sup>                | 0.06 | 0.72  | 95  | 95                       | 1.52                        |
| D<br>(Invention)  | (11)                                                                               | 2.2 × 10 <sup>-4</sup>                | 0.07 | 0.85  | 99  | 99                       | 1.64                        |
| E<br>(Comparison) | A-1                                                                                | 2.2 × 10 <sup>-6</sup>                | 0.05 | 0.45  | 26  | 26                       | 0.95                        |
| F                 | A-2                                                                                | 2.2 × 10 <sup>-5</sup>                | 0.07 | 0.62  | 51  | 51                       | 1.29                        |

TABLE 1-continued

| Sample            | Precursor Compound<br>of the Present<br>Invention or<br>Comparison<br>Antifoggants | Amount Added<br>(mol/m <sup>2</sup> ) | Fog  | Gamma | Relative*<br>Sensitivity | Maximum<br>Color<br>Density |
|-------------------|------------------------------------------------------------------------------------|---------------------------------------|------|-------|--------------------------|-----------------------------|
| (Comparison)<br>G | A-3                                                                                | $1.1 \times 10^{-5}$                  | 0.07 | 0.71  | 73                       | 1.27                        |
| (Comparison)      |                                                                                    |                                       |      |       |                          |                             |

\*Relative Sensitivity:

Relative sensitivity is shown by a reciprocal of an exposure amount required for obtaining a color density of fog + 0.2 and with the sensitivity of Control Sample A as 100.

As can be seen from the results shown in Table 1, in Samples B to D which contained the compounds of the present invention, generation of fog was depressed and the gamma, the sensitivity and the maximum color density were decreased very little.

### EXAMPLE 2

Sample B (present invention) and Sample G (containing the precursor for comparison) as described in Example 1 were stored for 1 week under the conditions of 40° C. and 80% RH and then subjected to the imagewise exposure and development processing in the same manner as in Example 1. As a result of these processings, Sample G showed remarkably low values of gamma, sensitivity and maximum color density, compared with Sample B. Accordingly, the precursor of the present invention has good storage stability, while the precursor used in Sample G lacks good stability because of a tendency for the blocking moiety to come off upon storage.

### EXAMPLE 3

To an aqueous solution containing 70 g of gelatin were simultaneously added at a constant rate an aqueous solution containing 1 kg of silver nitrate and an aqueous solution containing 210 g of potassium bromide and 290 g of sodium chloride over a period of 30 minutes. After removal of the soluble salts, gelatin was added to the emulsion. The resulting emulsion was subjected to gold sensitization and sulfur sensitization to obtain a silver chlorobromide emulsion (grain size: 0.27  $\mu\text{m}$ , bromide content: 30 mol %). To the emulsion was added 4-hydroxy-6-methyl-1,3,3a, 7-tetraazaindene as stabilizer.

Further, the blocked photographic agent (precursor) of the present invention, as set forth in Table 2 below, was added thereto. Subsequently, to the emulsion were added sodium 1-hydroxy-3,5-dichlorotriazine as hardener and sodium dodecylbenzenesulfonate as coating aid. The thus prepared emulsion was coated on a polyethylene terephthalate film at a silver coverage of 4.2 g/m<sup>2</sup>.

The film samples thus produced were exposed wedgewise using a xenon flash lamp for 10<sup>-5</sup> second, and developed with the developing solution shown below at 27° C. for 4 minutes, followed by stopping fixing, washing and drying. The densities of the thus processed samples were measured using a P-type densitometer (produced by Fuji Photo Film Co., Ltd.), and the sensitivity and fog values were measured. The standard point of optical density for determining the sensitivity was a point of fog + 0.5. The results obtained are shown in Table 2.

| 15 |  | Composition of the Developing Solution: |         |
|----|--|-----------------------------------------|---------|
|    |  | p-Methylaminophenol Sulfate             | 0.31 g  |
|    |  | Anhydrous Sodium Sulfite                | 39.6 g  |
|    |  | Hydroquinone                            | 6.0 g   |
|    |  | Anhydrous Sodium Carbonate              | 18.7 g  |
|    |  | Potassium Bromide                       | 0.86 g  |
|    |  | Citric Acid                             | 0.68 g  |
|    |  | Potassium Metahydrogensulfite           | 1.5 g   |
|    |  | Water to make                           | 1 liter |

| 25                |            | TABLE 2                           |      |                         |
|-------------------|------------|-----------------------------------|------|-------------------------|
| Sample            | Pre-cursor | Amount Added<br>(mol/kg emulsion) | Fog  | Relative<br>Sensitivity |
| 1<br>(Control)    | —          | —                                 | 0.07 | 100<br>(Standard)       |
| 2<br>(Invention)  | (1)        | $3.0 \times 10^{-4}$              | 0.05 | 96                      |
| 3<br>(Invention)  | (3)        | $3.0 \times 10^{-4}$              | 0.04 | 92                      |
| 4<br>(Invention)  | (4)        | $3.0 \times 10^{-4}$              | 0.05 | 97                      |
| 5<br>(Invention)  | (21)       | $3.0 \times 10^{-4}$              | 0.04 | 91                      |
| 6<br>(Comparison) | A-1        | $3.0 \times 10^{-4}$              | 0.05 | 46                      |

Comparison Compound A-1



As can be seen from the results shown in Table 2, the compounds of the present invention can depress the generation of fog accompanied by only a very slight decrease in sensitivity compared with Comparison Compound A-1.

### EXAMPLE 4

A silver halide emulsion containing 80 mol % of silver chloride, 19.5 mol % of silver bromide and 0.5 mol % of silver iodide was subjected to gold sensitization and sulfur sensitization. A mean grain size of silver halide grains in the emulsion was 0.31  $\mu\text{m}$ .

To each 1 kg portion of the silver halide emulsion were added the blocked photographic agent of the present invention as shown in Table 3 below, 0.1 g of 3-carboxymethyl-5-(3-ethyl-2-thiazolidinylideneethylidene)-rhodanine (spectral sensitizer), 0.18 g of 4-hydroxy-6-methyl-1,3,3a, 7-tetraazaindene (stabilizer), 0.45 g of

polyalkylene oxide compound (P-21), 1.2 g of sodium dodecylbenzenesulfonate (surface active agent), 0.48 g of mucochloric acid (hardener) and 30 g of a polymer latex as described in Japanese Patent Publication No. 5331/70. The thus prepared emulsion was coated on a polyethylene terephthalate film at a silver coverage of 3.9 g/m<sup>2</sup> to produce a photographic material.

The samples thus produced were contacted with a gray contact screen for negative (150 L/inch, produced by Dai-Nippon Screen Co., Ltd.) and exposed to tungsten light (color temperature of 5,400° K.) for 1 second through a step wedge having a difference of 0.1 (log E) in each step. Then, the samples were developed with the lith type developing solution shown below at 27° C. for 100 seconds using an automatic developing machine, stopped, fixed, washed, and dried.

Composition of the Developing Solution:

|                                      |          |
|--------------------------------------|----------|
| Hydroquinone                         | 15 g     |
| Formaldehyde-Sodium Hydrogensulfite  | 50 g     |
| Adduct                               |          |
| Potassium Carbonate                  | 30 g     |
| Sodium Sulfite                       | 2.5 g    |
| Potassium Bromide                    | 2.0 g    |
| Boric Acid                           | 5.0 g    |
| Sodium Hydroxide                     | 3.0 g    |
| Triethylene Glycol                   | 40 g     |
| Disodium Ethylenediaminetetraacetate | 1.0 g    |
| Water to make                        | 1,000 cc |

The samples thus processed were measured with regard to dot areas of 10%, 50% and 90%, respectively. The sensitivities of the samples were compared by a reciprocal of an exposure amount required for obtaining the dot area of 50%. In addition, the screen range was determined from the difference between the logarithm of the exposure amount providing a dot area of 10% and that of an exposure amount providing a dot area of 90%. The results obtained are shown in Table 3.

TABLE 3

| Sample         | Pre-cursor | Amount<br>Added<br>(mol/kg<br>emulsion) | Sensitivity<br>(Standard) | Fog  | Screen<br>Range |
|----------------|------------|-----------------------------------------|---------------------------|------|-----------------|
| 1 (Control)    | —          | —                                       | 100                       | 0.06 | 0.9             |
| 2 (Invention)  | (1)        | 2.0 × 10 <sup>-4</sup>                  | 97                        | 0.04 | 1.1             |
| 3 (Invention)  | (1)        | 4.0 × 10 <sup>-4</sup>                  | 92                        | 0.04 | 1.0             |
| 4 (Comparison) | A-1        | 2.0 × 10 <sup>-4</sup>                  | 47                        | 0.04 | 1.0             |
| 5 (Comparison) | A-1        | 4.0 × 10 <sup>-4</sup>                  | 36                        | 0.04 | 1.1             |
| 6 (Invention)  | (30)       | 2.0 × 10 <sup>-4</sup>                  | 96                        | 0.04 | 1.1             |
| 7 (Invention)  | (30)       | 4.0 × 10 <sup>-4</sup>                  | 91                        | 0.04 | 1.2             |
| 8 (Comparison) | A-4        | 2.0 × 10 <sup>-4</sup>                  | 50                        | 0.04 | 1.1             |
| 9 (Comparison) | A-4        | 4.0 × 10 <sup>-4</sup>                  | 33                        | 0.04 | 1.2             |

Comparison Compound A-4



As can be seen from the results shown in Table 3, the compounds of the present invention can depress the generation of fog without being attended by a substantial decrease in the sensitivity. Also, the compounds of the present invention can produce an improvement in screen range without being attended by a substantial decrease in the sensitivity.

While the invention has been described in detail and with reference to specific embodiments thereof, it will be apparent to one skilled in the art that various changes and modifications can be made therein without departing from the spirit and scope thereof.

What is claimed is:

1. A silver halide photographic material which comprises a support having coated thereon a light-sensitive silver halide emulsion layer, wherein the photographic material contains a blocked photographic agent represented by the following general formula (I):



20 wherein A represents a photographic agent moiety which is bonded to a blocking moiety through a hetero atom, or a precursor thereof; R<sup>1</sup> represents a hydrogen atom or a substituent group; and Z represents atoms necessary to form a carbocyclic ring or a heterocyclic ring, wherein A is a group represented by the following general formula (II)



30 wherein B represents a photographic agent moiety selected from the group consisting of an antifoggant, a development inhibitor, a developing agent selected from the group consisting of p-phenylenediamines, hydroquinones, a pyrazolidone, a fogging agent and a dyer, a bleach accelerating agent, which is bonded to X through a hetero atom contained in B; X represents a divalent linkage group which is bonded to a blocking moiety through a hetero atom contained in X; and m is 0 or 1, wherein the photographic agent moiety represented by B is directly bonded to the blocking moiety through a hetero atom contained in B.

35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 87

droquinones, a pyrazolidone, a fogging agent, and a dye, a bleach accelerating agent, which is bonded to X through a hetero atom contained in B; X represents a divalent linkage group which is bonded to a blocking moiety through a hetero atom contained in X; and m is 0 or 1, wherein the photographic agent moiety represented by B is bonded to the divalent linkage group represented by X through a hetero atom contained in B.

3. A silver halide photographic material as in claim 1 or 2, wherein the blocked photographic agent is an antifoggant and the blocked photographic agent is contained in the photographic material in an amount of 10<sup>-8</sup> to 10<sup>-1</sup> mol per mol of silver in the silver halide emulsion.

4. A silver halide photographic material as in claim 1 or 2, wherein the blocked photographic agent is a development inhibitor and the blocked photographic agent is contained in the photographic material in an amount of 10<sup>-8</sup> to 10<sup>-1</sup> mol per mol of silver in the silver halide emulsion.

5. A silver halide photographic material as in claim 1 or 2, wherein the blocked photographic agent is an auxiliary developer of a pyrazolidone type and the blocked photographic agent is contained in the photographic material in an amount of 10<sup>-4</sup> to 10 mol per mol of silver in the silver halide emulsion.

6. A silver halide photographic material as in claim 1 or 2, wherein the blocked photographic agent is a fogging agent and the blocked photographic agent is contained in the photographic material in an amount of 10<sup>-2</sup> to 10<sup>-6</sup> mol per mol of silver in the silver halide emulsion.

7. A silver halide photographic material as in claim 1 or 2, wherein the blocked photographic agent is a bleach accelerating agent and the blocked photographic agent is contained in the photographic material in an amount of 10<sup>-5</sup> to 10<sup>-1</sup> mol per mol of silver in the silver halide emulsion.

8. A silver halide photographic material as in claim 1 or 2, wherein the blocked photographic agent is a dye and the blocked photographic agent is contained in an amount of 10<sup>-3</sup> to 1 mol per mol of silver in the silver halide emulsion.

9. A silver halide photographic material which comprises a support having coated thereon a light-sensitive silver halide emulsion layer, wherein the photographic material contains a blocked photographic agent represented by the following general formula (I):



wherein A represents a photographic agent moiety which is bonded to a blocking moiety through a hetero atom, or a precursor thereof; R<sup>1</sup> represents a hydrogen atom or a substituent group; and Z represents atoms necessary to form a carbocyclic ring or a heterocyclic ring, wherein A is a group represented by the following general formula (II):



wherein B represents a photographic agent moiety selected from the group consisting of mercaptotetrazoles, mercaptotriazoles, mercaptopyrimidines, mercaptoben-

zimidazoles, mercaptotimidazoles, mercaptobenzoxazoles, mercaptobenzthiazoles, mercaptothiadiazoles, benzotriazoles and indazoles which is bonded to X through a hetero atom contained in B; X represents a divalent linkage group which is bonded to a blocking moiety through a hetero atom contained in X; and m is 0 or 1, wherein the photographic agent moiety represented by B is bonded to the divalent linkage group represented by X through a hetero atom contained therein.

10. A silver halide photographic material which comprises a support having coated thereon a light-sensitive silver halide emulsion layer, wherein the photographic material contains a blocked photographic agent represented by the following general formula (I):



wherein A represents a photographic agent moiety which is bonded to a blocking moiety through a hetero atom, or a precursor thereof; R<sup>1</sup> represents a hydrogen atom or a substituent group; and Z represents atoms necessary to form a carbocyclic ring or a heterocyclic ring, wherein A is a group represented by the following general formula (II):



wherein B represents a photographic agent moiety selected from pyrazolidones which is bonded to X through a hetero atom contained in B; X represents a divalent linkage group which is bonded to a blocking moiety through a hetero atom contained in X; and m is 0 or 1, wherein the photographic agent moiety represented by B is bonded to the divalent linkage group represented by X through a hetero atom contained therein.

11. A silver halide photographic material which comprises a support having coated thereon a light-sensitive silver halide emulsion layer, wherein the photographic material contains a blocked photographic agent represented by the following general formula (I):



wherein A represents a photographic agent moiety which is bonded to a blocking moiety through a hetero atom, or a precursor thereof; R<sup>1</sup> represents a hydrogen atom or a substituent group; and Z represents atoms necessary to form a carbocyclic ring or a heterocyclic ring, wherein A is a group represented by the following general formula (II):



wherein B represents a photographic agent moiety selected from the group consisting of hydrazines and hydrazides which is bonded to X through a hetero atom

contained in B; X represents a divalent linkage group which is bonded to a blocking moiety through a hetero atom contained in X; and m is 0 or 1, wherein the photographic agent moiety represented by B is bonded to the divalent linkage group represented by X through a hetero atom contained therein.

12. A silver halide photographic material which comprises a support having coated thereon a light-sensitive silver halide emulsion layer, wherein the photographic material contains a blocked photographic agent represented by the following general formula (I):



wherein A represents a photographic agent moiety which is bonded to a blocking moiety through a hetero atom, or a precursor thereof; R<sup>1</sup> represents a hydrogen atom or a substituent group; and Z represents atoms necessary to form a carbocyclic ring or a heterocyclic ring, wherein A is a group represented by the following general formula (II):



wherein B represents sodium thiosulfate as a photographic agent moiety which is bonded to X through a hetero atom contained in B; X represents a divalent linkage group which is bonded to a blocking moiety through a hetero atom contained in X; and m is 0 or 1, wherein the photographic agent moiety represented by B is bonded to the divalent linkage group represented by X through a hetero atom contained therein.

13. A silver halide photographic material which comprises a support having coated thereon a light-sensitive silver halide emulsion layer, wherein the photographic material contains a blocked photographic agent represented by the following general formula (I):



5 wherein A represents a photographic agent moiety which is bonded to a blocking moiety through a hetero atom, or a precursor thereof; R<sup>1</sup> represents a hydrogen atom or a substituent group; and Z represents atoms necessary to form a carbocyclic ring or a heterocyclic ring, wherein A is a group represented by the following general formula (II):



10 wherein B represents a photographic agent moiety selected from aminoalkylthiols which is bonded to X through a hetero atom contained in B; X represents a divalent linkage group which is bonded to a blocking moiety through a hetero atom contained in X; and m is 0 or 1, wherein the photographic agent moiety represented by B is bonded to the divalent linkage group represented by X through a hetero atom contained therein.

14. A silver halide photographic material which comprises a support having coated thereon a light-sensitive silver halide emulsion layer, wherein the photographic material contains a blocked photographic agent represented by the following general formula (I):



20 wherein A represents a photographic agent moiety which is bonded to a blocking moiety through a hetero atom, or a precursor thereof; R<sup>1</sup> represents a hydrogen atom or a substituent group; and Z represents atoms necessary to form a carbocyclic ring or a heterocyclic ring, wherein A is a group represented by the following general formula (II):



25 wherein B represents a photographic agent moiety selected from the group consisting of azo dyes and azomethine dyes which is bonded to X through a hetero atom contained in B; X represents a divalent linkage group which is bonded to a blocking moiety through a hetero atom contained in X; and m is 0 or 1, wherein the photographic agent moiety represented by B is bonded to the divalent linkage group represented by X through a hetero atom contained therein.

\* \* \* \* \*